

Jan. 18, 1938.

I. J. B. DEMERS

2,105,906

METHOD OF HOT PLATING CONTAINERS

Filed Oct. 26, 1936

*Fig. 1*



*Fig. 2*



*Fig. 3*



Inventor

Isaie J. B. Demers

By *Stupack & Stupack*  
Attorneys

## UNITED STATES PATENT OFFICE

2,105,906

## METHOD OF HOT PLATING CONTAINERS

Isaie J. B. Demers, St. Paul, Minn., assignor to  
 Superior Metal Products Company, St. Paul,  
 Minn., a corporation of Delaware

Application October 26, 1936, Serial No. 107,601

7 Claims. (Cl. 91—70.2)

It is an object of this invention to provide a novel process for hot plating the walls and bottoms of containers simultaneously and in such manner that the thickest plating is located on the bottoms and adjacent parts which are subjected to the most harmful wear and corroding influences.

A further object is to provide a novel process for obtaining improved distribution of the plating material on a container having a closed bottom and at the same time to eliminate waste of plating material by avoiding unnecessary thickness of plating and accidental spilling of the plating.

Other objects will appear and be more fully pointed out in the following specification and claims.

In the manufacture of many types of sheet metal containers, such for example as those used for dairy products, it is desirable, in the interest of economy and to avoid unsightly and unsanitary joints, to weld the bottoms to the walls before the plating operation. When this is done, however, the problem of obtaining the proper distribution of the plating material to impart maximum durability to the container is rendered more difficult, particularly where the finished containers have no bottom opening which can be utilized as an outlet for the excess of plating material during the plating process. One method of solving this problem is described and claimed in my Patent No. 2,018,951, dated October 29, 1935. By the method described and claimed herein I eliminate the necessity for an opening or perforation in the bottom of the container and at the same time secure the advantages of increased thickness of plating material on the bottom and lower portions of the walls of the containers.

My improved method and suitable apparatus for practicing it is illustrated in the accompanying drawing in which,

Figure 1 is a central, vertical section through a container and listing table supporting the container and also illustrating a device for removing the excess of plating material;

Fig. 2 is a larger vertical section through the bottom portions of the container and removing device, and

Fig. 3 illustrates the method of emptying the removing device.

In the drawing, a milk can is indicated generally by the numeral 4. The principal parts of this can are assembled in the usual or suitable manner, preferably by welding the top portions

and bottom 5 to the cylindrical walls 6. The bottom 5 is internally concave in shape and a small indentation 7 is preferably formed centrally therein to facilitate removal of the excess plating material, as hereinafter described.

As a preliminary to the plating or tinning of the containers, the latter are thoroughly cleansed, usually in an acid bath. The entire container is now immersed in a bath of the molten plating metal so that the latter completely covers the inner and outer surfaces of the container. Two or more immersions in the plating material are usually required. After the final immersion in the plating material, the greater part of the excess from the interior surfaces is decanted from the top and then the container is supported in upright position, as indicated in Figs. 1 and 2 of the drawing while the plating cools and hardens.

During this step of the process containers are usually placed on a "listing" plate 8, shown diagrammatically in Fig. 1. This plate is supported in horizontal position in the top of a kettle or vat 9 containing a body of the plating material which is maintained in its molten condition by heating. Suitable burners are well known in this art and are shown diagrammatically in the drawing, being indicated by the numeral 10. The surface of the metal is maintained slightly above the plate 8 so that the lower extremity of the container 4 rests in the hot metal while the excess of plating material from the exterior of the container flows into the vat 9.

While thus positioned on the listing plate, the container cools progressively from the top down and the excess of plating material from the interior surfaces collects in a small pool, indicated by the numeral 11 in Fig. 2, on the bottom in and around the depression 7. While this pool is still molten, it is removed directly upward so as not to spread or spill the metal on the solidified coating elsewhere on the container. Finally, when the container is sufficiently cool for removal from the listing plate, the entire surfaces are smoothly plated without excess or irregular deposits and the desired maximum thickness of plating on the bottom and adjacent parts is obtained.

To facilitate the removal of the pool 11 of molten metal, I provide a small receptacle 12 mounted on a pipe 13 and formed with a passage 14 terminating in a short nipple 15 at its lower end. This passage communicates with the interior of the receptacle 12 at a point spaced upward from the bottom of said receptacle. By

this arrangement, a quantity of molten metal 16 may be trapped in the receptacle 12 for removal from the container 4. The pipe 13 communicates at its upper end with a hose 17 connected 5 to a vacuum tank or other device for exhausting air from the receptacle 12. The application of the reduced pressure may be controlled by a valve 18. The passage 14 is preferably located at one side of the receptacle 12 to facilitate the discharge of the metal 16 from the receptacle. As 10 illustrated in Fig. 3, the device when not in use is preferably placed on its side so that the metal 16 flows out through the passage 14 and should be kept hot between operations by supporting it 15 above or in a flame. A burner 19 for heating the receptacle 12 is indicated in Fig. 3. The pool of coating material 11 may be quickly removed, at the proper time as hereinbefore described, merely by lowering the receptacle 12 into 20 the container and submerging the tip of the nipple 15 in the pool, while the vacuum is applied through the pipe 13 and hose 17. The receptacle 12 is then withdrawn from the container and emptied. By my arrangement of the passage 25 14, the molten plating material is trapped in the receptacle 12 and there is no dripping or other defacing of the hardened plating as the device is withdrawn from the container. Between operations, the receptacle 12 is placed on its side, as 30 indicated in Fig. 3, to empty the coating material through the passage 14.

By reason of the cooling in upright position and fact that the lower portions of the container 4 retain the heat longest, I secure smooth plating 35 20 on the walls 6 and bottom 5 which is progressively thicker from the top down. This is the condition desired because it affords the maximum protection when needed and an unusually durable container results.

40 My improved method may be employed in applying numerous plating materials, such as zinc or other galvanizing metals, as well as tin and other platings which are applied in a molten condition to various articles of manufacture, including tanks and cans of various types.

Having described my invention, what I claim as new and desire to protect by Letters Patent is:

1. The method of hot plating a container having an imperforate bottom which consists in 50 applying a coating of molten plating material to said container, then placing it in such position as to accumulate a pool of excess coating material on said bottom while allowing said container to cool progressively from the top down and then removing said pool from above while in 55 molten condition.

2. The method of hot plating a container to effect progressively increasing thickness of plating material toward the bottom which consists 60

in securing to the walls of the container an imperforate bottom, then hot plating said container, then accumulating an excess of coating material on said bottom while allowing said container to partially cool and then removing said excess of plating material from above while in molten condition. 5

3. The method of hot plating a container having a bottom and walls which consists in applying a coating of molten plating material to said 10 walls and bottom and then placing the container in such position as to accumulate the excess of coating material from the interior surfaces on said bottom while allowing said container to cool partially and then removing said 15 excess of plating material by drawing it directly upward while in molten condition.

4. The method of hot plating a cylindrical container having an internally concave bottom which 20 consists in immersing said container in hot plating material, then placing it in upright position and accumulating a quantity of the excess plating material on said bottom while allowing the container to cool progressively from the top down and then removing said excess of plating material 25 from above while in molten condition and while retaining said container in substantially upright position.

5. The method of hot plating a container having an internally concave bottom which consists 30 in immersing said container in hot plating material, then placing it in such position as to accumulate the excess of plating material from the interior surfaces of the container in a pool on the inner surface of said bottom while allowing the 35 container to partially cool and then removing said excess of plating material from above, while retaining said container in said position.

6. The method of hot plating a container which 40 consists in forming in the inner surface of the bottom of said container an indentation, then hot plating said container and placing it in such position as to collect the excess of the liquid contents in and around said indentation and then allowing the container to cool progressively from 45 the top down while withdrawing said excess of plating material from above and retaining said container in said position until the plating has hardened.

7. The method of hot plating a container which 50 consists in forming in the inner surface of the bottom of said container an indentation, then hot plating said container and placing it in such position as to collect the excess of the liquid contents in and around said indentation while allowing the container to partially cool, then withdrawing said excess of plating material from said 55 indentation while retaining said container in said position.